# EUROPEAN PATENT APPLICATION

(11) **EP 4 640 880 A1**
(43) Date of publication of application: **29.10.2025**
(21) Application number: 23907567.4
(22) Date of filing: 13.12.2023
(51) Int. Cl.: C22C 38/04, C22C 38/02, C22C 38/06, C22C 38/00, C21D 8/02, B21C 47/02, C21D 9/46

(54) **HIGH-STRENGTH STEEL SHEET AND MANUFACTURING METHOD THEREFOR**

(30) Priority: 21.12.2022 KR 20220180619
(71) Applicant: POSCO Co., Ltd, Pohang-si, Gyeongsangbuk-do 37859 (KR)
(72) Inventor: PARK, Kyong-Su, Pohang-si Gyeongsangbuk-do 37859 (KR)
(74) Representative: Meissner Bolte Partnerschaft mbB
(86) International application number: PCT/KR2023/020553
(87) International publication number: WO 2024/136281

(57) **Abstract**

Disclosed are: a high-strength steel sheet having excellent tensile strength and yield strength by including 90 area% or more of a martensite microstructure via rapid cooling of a hot-rolled steel sheet immediately after hot-rolling, under a rapid cooling condition; and a manufacturing method for the steel sheet. The steel sheet according to the present invention comprises, by weight %, 0.11 to 0.30% of C, 0.10 to 3.00% of Mn, more than 0% to 0.50% or less of Si, more than 0% to 0.10% or less of Al, more than 0% to 0.05% or less of P, more than 0% to 0.03% or less of **S,** more than 0% to 0.03% or less of N, and the remainder of Fe and other unavoidable impurities, and comprises, with respect to a total of 100 area%, 90 to 100 area% of the martensite microstructure.

## Description

### FIELD

The present disclosure relates to a high-strength steel plate and a method for manufacturing the same, and more specifically, to a high-strength steel plate having excellent tensile strength and yield strength, including 90 area% or greater of martensite, by rapidly cooling a hot-rolled steel plate immediately after the hot rolling without adding a large amount of carbon or manganese to an alloy composition, and a method for manufacturing the same.

### DESCRIPTION OF RELATED ART

Steel plates are widely used in all industrial fields, and are mainly used as materials for automobile parts and industrial parts that are subject to repeated stress or deformation.

Among the steel plates, high-carbon steel plates are widely used for various parts because of their strength. Examples of automobile parts that use the high-carbon steel plates include clutch parts, seat belt spring parts, or the like. Examples of industrial parts that use the high-carbon steel plates include industrial spring parts, tool parts, or the like.

When manufacturing such high-carbon steel, heat treatment is generally performed after hot rolling or cold rolling to secure desired materiality.

To manufacture the high-carbon steel plate with excellent durability, a method for manufacturing spring steel via a quenching process and a heat treatment process, a method for securing a martensite structure via high-temperature heat treatment after cold rolling, a method for increasing a strength of the spring steel via an induction heat treatment process, and the like are being studied.

However, in connection with the recent rapid climate change, carbon neutrality has emerged as an important issue across all industries, and a reduction in carbon emissions is also required in a steel industry without exception.

Accordingly, attempts are being made to reduce the carbon emissions by lowering a carbon content in an alloy composition or controlling heat treatment process conditions.

### DISCLOSURE

### TECHNICAL PURPOSE

The present disclosure is to provide a high-strength steel plate having excellent tensile strength and yield strength.

In addition, the present disclosure is to provide a high-strength steel plate that may be applied to automobile parts, industrial parts, and the like.

In addition, the present disclosure is to provide a method for manufacturing a high-strength steel plate having excellent eco-friendly characteristics by reducing a manufacturing cost and carbon emissions.

Purposes of the present disclosure are not limited to the purposes mentioned above, and other purposes and advantages of the present disclosure that are not mentioned may be understood by the following description and will be more clearly understood by embodiments of the present disclosure. In addition, it will be easily understood that the purposes and advantages of the present disclosure may be realized by means and combinations thereof indicated in the patent claims.

### TECHNICAL SOLUTION

A steel plate according to the present disclosure includes, in weight%, C: 0.1 1 to 0.30%, Mn: 0.10 to 3.00%, Si: greater than 0% and equal to or smaller than 0.50%, Al: greater than 0% and equal to or smaller than 0.10%, P: greater than 0% and equal to or smaller than 0.05%, S: greater than 0% and equal to or smaller than 0.03%, N: greater than 0% and equal to or smaller than 0.03%, remainder Fe and other inevitable impurities, and has a martensite microstructure of 90 to 100 area% with respect to a total 100 area%.

The steel plate may further include B: 0.0003 to 0.005wt%.

When a packet of the martensite having a long axis direction aligned within 45° from a rolling direction is called martensite elongated along the rolling direction, an area percentage of the martensite elongated along the rolling direction in the martensite may be equal to or greater than 60%. Further, an area percentage of packets having a long axis to a short axis ratio equal to or greater than 2:1 in the martensite may be equal to or greater than 50%.

The steel plate may include 0 to 10 area% of microstructures of one or more of ferrite and retained austenite with respect to the total 100 area%. Further, the steel plate may include 0 to 5 area% of microstructures of one or more of pearlite and bainite with respect to the total 100 area%.

A tensile strength may be equal to or greater than 1800 MPa and a yield strength may be equal to or greater than 1700 MPa.

Particularly, when C is in a range of 0.18 to 0.30%, a tensile strength may be equal to or greater than 1910 MPa and a yield strength may be equal to or greater than 1880 MPa.

A yield strength (MPa) and alloying elements (%) of the steel plate may satisfy following Relational Expression 1. Relational Expression 1:[yield strength/{C+(Mn×0.05)}]≥6,000

A method for manufacturing a steel plate according to the present disclosure includes (a) heating a slab including, in wt%, C: 0.11 to 0.30%, Mn: 0.10 to 3.00%, Si: greater than 0% and equal to or smaller than 0.50%, Al: greater than 0% and equal to or smaller than 0.10%, P: greater than 0% and equal to or smaller than 0.05%, S: greater than 0% and equal to or smaller than 0.03%, N: greater than 0% and equal to or smaller than 0.03%, remainder Fe and other unavoidable impurities, (b) hot-rolling the heated slab, (c) rapidly cooling the hot-rolled slab at a cooling rate of 50 to 1000°C/sec within 5 seconds after the hot rolling and then coiling the cooled slab, and (d) cold-rolling the slab after the coiling.

In the (a), the heating may be performed at 1050 to 1350°C.

In the (b), the hot rolling may be performed at 800 to 950°C.

In the (c), each of the rapid cooling and the coiling may be performed at 100 to 350°C.

In the (d), the cold rolling may be performed at a reduction percentage of 50 to 80%.

### TECHNICAL EFFECT

The high-strength steel plate according to the present disclosure has the excellent tensile strength and yield strength, including 90 area% or greater of the martensite microstructure, by cooling the hot-rolled steel plate immediately after the hot rolling under the rapid cooling conditions without adding the large amount of carbon or manganese to the alloy composition.

In particular, even though the heat treatment is omitted immediately after the hot rolling and immediately after the cold rolling, martensite formed by the rapid cooling has the form that is elongated by the cold rolling, so that the strength of the steel plate is significantly improved.

In addition, not only may the energy and the manufacturing cost required for manufacturing the steel plate be reduced, but also the carbon emissions during the high-temperature heat treatment process may be reduced, thereby securing the eco-friendly characteristics. In addition, the manufactured steel plate may exhibit the high strength, so that it may be applied to the automotive parts such as the clutch parts and the industrial spring parts, and the industrial parts such as the spring parts and the tool parts.

In addition to the effects described above, specific effects of the present disclosure will be described together with specific details for carrying out the invention below.

### BRIEF DESCRIPTION OF DRAWINGS

FIG. 1 is a flowchart showing a method for manufacturing a high-strength steel plate according to the present disclosure.
FIG. 2 is a photograph showing a 100 area% martensite microstructure before cold rolling according to the present disclosure.
FIG. 3 is a photograph showing a martensite microstructure after cold rolling with a 70% reduction percentage according to the present disclosure.

### DETAILED DESCRIPTIONS

The above-mentioned purposes, features, and advantages will be described in detail later with reference to the attached drawings, so that those skilled in the art in the technical field to which the present disclosure belongs may easily practice the technical ideas of the present disclosure. In describing the present disclosure, when it is determined that a detailed description of the publicly known technology related to the present disclosure may unnecessarily obscure the gist of the present disclosure, the detailed description thereof will be omitted. Hereinafter, a preferred embodiment according to the present disclosure will be described in detail with reference to the attached drawings. In the drawings, identical reference numerals are used to indicate identical or similar components.

Hereinafter, it may mean that when a first component is described to be disposed "on (or under)" a second component, the first component may not only be disposed in contact with a top surface (or a bottom surface) of the second component, but also be disposed on the second component with a third component interposed therebetween.

Additionally, it should be understood that when a component is described as being "connected to", "combined to", or "coupled to" another component, the components may be directly connected or coupled to each other, but other components may be "interposed" therebetween and the components may be "connected to", "combined to", or "connected to" each other via said other components.

Hereinafter, a high-strength steel plate and a method for manufacturing the same according to some embodiments of the present disclosure will be described.

The present inventor studied the steel plate for application to high-carbon parts such as an industrial spring.

At first, carbon and manganese were added in large amounts to an alloy composition to increase a strength of the steel plate. It was identified that adding the large amounts of carbon and manganese to the alloy composition exhibited high-strength, but weldability and formability deteriorated, and there was a cost burden in an economical aspect because of a high cost of manganese. In addition, it was found that, when heat treatment was performed immediately after hot rolling and then the heat-treated hot-rolled steel plate was cold-rolled and then subjected to quenching heat treatment as in an existing steel plate manufacturing method, carbon emissions were great during the high-temperature heat treatment process.

To solve such problems, the present inventor lowered a carbon content to 0.30% or lower and a manganese content to 3.0% or lower, and controlled process conditions.

In the process conditions, the high-temperature heat treatment was omitted, and rapidly cooling was performed at a cooling rate of 50 to 1000°C/sec within 5 seconds immediately after the hot rolling to secure martensite of a hard structure by 90 area% or more, so that high tensile strength and yield strength were able to be exhibited simultaneously.

Furthermore, by controlling martensite to have an elongated form by the cold rolling, an effect of further improving the strength of the steel plate was identified.

Accordingly, the present inventor was able to manufacture the high-strength steel plate that may effectively improve a strength of automobile parts and industrial parts by omitting the high-temperature heat treatment and controlling the cooling conditions of the hot-rolled steel plate without adding the large amount of carbon or manganese to the alloy composition.

The high-strength steel plate manufactured according to the present disclosure may exhibit materiality effects of tensile strength equal to or greater than 1800MPa and yield strength equal to or greater than 1700MPa, as well as environmental friendliness resulted from the reduced carbon content.

The steel plate according to the present disclosure may contain, in wt%, C: 0.11 to 0.30%, Mn: 0.10 to 3.00%, Si: greater than 0% and equal to or smaller than 0.50%, Al: greater than 0% and equal to or smaller than 0.10%, P: greater than 0% and equal to or smaller than 0.05%, S: greater than 0% and equal to or smaller than 0.03%, N: greater than 0% and equal to or smaller than 0.03%, remainder Fe and other inevitable impurities, and may further contain B: 0.0003 to 0.005wt%.

Further, the steel plate includes 90 to 100 area% of martensite microstructure with respect to a total 100 area%.

Hereinafter, unless otherwise specified, the % indicating a content of each element is based on wt%.

### Carbon (C): 0.11 to 0.30%

Carbon (C) is an element that effectively contributes to improving the strength of steel, so that, in the present disclosure, a certain level or more of carbon (C) may be included to secure the strength of the steel plate.

When the carbon (C) content is not at the certain level, a large number of low-temperature structures such as pearlite and bainite are formed during the cooling after the hot rolling, so that a microstructure that the present disclosure aims for may not be secured. Regarding a lower limit, the carbon (C) content may be equal to or greater than 0.110%. Preferably, it may be equal to or greater than 0.150%, and more preferably, may be equal to or greater than 0.200% or greater than 0.200%.

On the other hand, when carbon (C) is added excessively, the strength of the steel may be improved, but cold-rollability may be reduced. Regarding an upper limit, the carbon (C) content may be equal to or smaller than 0.300%, and preferably, may be equal to or smaller than 0.295%.

In particular, when the alloy composition satisfies C: 0.18 to 0.30%, the steel plate may have the tensile strength (TS) equal to or greater than 1910 MPa and the yield strength (YS) equal to or greater than 1880 MPa.

### Manganese (Mn): 0.10 to 3.00%

Manganese (Mn) is an element that effectively contributes to improving the strength and hardenability of the steel. In addition, manganese (Mn) forms MnS by combining with sulfur (S), which is inevitably introduced during the steel manufacturing process, and is therefore an element that effectively prevents cracking caused by sulfur (S).

To achieve such an effect, regarding a lower limit, the manganese (Mn) content may be equal to or greater than 0.10%. A preferable manganese (Mn) content may be equal to or greater than 0.300%, and a more preferable manganese (Mn) content may be equal to or greater than 0.500%.

On the other hand, when manganese (Mn) is added excessively, there is concern about a decrease in the tensile strength because of retained austenite, and it is not desirable in terms of economic efficiency. Therefore, regarding an upper limit, the manganese (Mn) content may be equal to or smaller than 3.00%. Preferably, it may be equal to or smaller than 2.90%, and more preferably, may be equal to or smaller than 2.80%.

### Silicon (Si): greater than 0% and equal to or smaller than 0.50%

Silicone (Si) is an element with a strong affinity for oxygen, so that when added in a large amount, it may cause a deterioration of a surface quality caused by surface scale, and it may also be not preferable in terms of the weldability. Therefore, regarding an upper limit, the silicon (Si) content may be equal to or smaller than 0.50%, and preferably, may be equal to or smaller than 0.45%.

In one example, because silicon (Si) not only acts as a deoxidizer but also is an element that contributes to improving the strength of the steel, in the present disclosure, addition of silicon (Si) is not completely excluded and thus 0% is able to be excluded from a lower limit of the content thereof. A lower limit of a preferable silicon (Si) content may be equal to or greater than 0.03%.

### Aluminum (Al): greater than 0% and equal to or smaller than 0.10%

Aluminum (Al) is an element that combines with oxygen in the steel and acts as a deoxidizer. In the present disclosure, for such an effect, aluminum (Al) may be added, and 0% may be excluded from a lower limit of the content thereof. A lower limit of a preferable aluminum (Al) content may be equal to or greater than 0.01%.

On the other hand, when aluminum (Al) is added excessively, not only will inclusions increase, but workability of the steel plate may also be reduced. Regarding an upper limit, the aluminum (Al) content may be equal to or smaller than 0.10%, and preferably, may be equal to or smaller than 0.08%.

### Phosphorus (P): greater than 0% and equal to or smaller than 0.05%

Phosphorus (P) is a major element that segregates at a grain boundary and causes a decrease in toughness of the steel, so that it is desirable to control the phosphorus (P) content as low as possible. Therefore, it is theoretically advantageous to set the phosphorus (P) content to 0%. However, phosphorus (P) is an impurity that is inevitably introduced during the steelmaking process, and controlling the phosphorus (P) content to 0% is able to cause an excessive process load.

Considering this, the phosphorus (P) content may be greater than 0% and equal to or smaller than 0.05%, and preferably, may be greater than 0% and equal to or smaller than 0.03%.

### Sulfur (S): greater than 0% and equal to or smaller than 0.03%

Sulfur (S) is an element that forms MnS, increases an amount of precipitates, and embrittles the steel, so that it is desirable to control the sulfur (S) content as low as possible. Therefore, it is theoretically advantageous to limit the sulfur (S) content to 0%. However, sulfur (S) is also an impurity that is inevitably introduced during the steelmaking process, and controlling the content thereof to 0% is able to cause the excessive process load.

Considering this, the sulfur (S) content may be greater than 0% and equal to or smaller than 0.03%, and preferably may be greater than 0% and equal to or smaller than 0.01%.

### Nitrogen (N): greater than 0% and equal to or smaller than 0.03%

Because nitrogen (N) is an element that causes cracks in a slab by forming nitrides during continuous casting, it is desirable to control the content thereof as low as possible. Therefore, it is theoretically advantageous to limit the nitrogen (N) content to 0%. However, nitrogen (N) is also an impurity that is inevitably introduced during the steelmaking process, and controlling the content thereof to 0% is able to cause the excessive process load. Considering this, the nitrogen (N) content may be greater than 0% and equal to or smaller than 0.03%, and preferably, may be greater than 0% and equal to or smaller than 0.01%.

### Boron (B): 0.0003 to~ 0.005wt%

Boron (B) is an element that effectively contributes to improving the hardenability of the steel. Even with a small amount of addition, boron (B) is an element that may effectively suppress transformation into the low-temperature structure such as ferrite and pearlite during the cooling after the hot rolling.

To achieve such an effect, regarding a lower limit, the boron (B) content may be equal to or greater than 0.0003%, and preferably, may be equal to or greater than 0.001%.

On the other hand, when boron (B) is added excessively, boron (B) may react with iron (Fe) and cause grain boundary embrittlement. Regarding an upper limit, the boron (B) content may be equal to or smaller than 0.005%, and preferably, may be equal to or smaller than 0.0045%.

The steel plate of the present disclosure may contain remainder Fe and other inevitable impurities in addition to the aforementioned components. However, because unintended impurities may inevitably be mixed from a raw material or a surrounding environment during the normal manufacturing process, the unintended impurities are not able to be completely excluded. Because such impurities are known to anyone with ordinary knowledge in the present technical field, not all of them are specifically mentioned in the present document. In addition, additional addition of effective components other than the aforementioned components is not completely excluded.

Hereinafter, the microstructure included in the steel plate of the present disclosure will be described in more detail.

The steel plate of the present disclosure includes martensite as a matrix structure. A fraction of martensite may be 90 to 100 area% relative to the total 100 area% of the steel plate, and preferably 95 to 100 area%. Because the steel plate of the present disclosure includes martensite, which is a hard structure, as the matrix structure, high strength and yield ratio may be secured at the same time.

Martensite included in the steel plate of the present disclosure is formed by the rapid cooling after the hot rolling and is elongated by the subsequent cold rolling, so that an area percentage of martensite elongated along a rolling direction in entire martensite included in the steel plate may be 60 to 100%, and preferably may be 80 to 95%.

In this regard, martensite elongated along the rolling direction means that a long axis direction of a martensite packet is aligned within 45° from the rolling direction, and preferably means that the long axis direction of the packet is aligned parallel to the rolling direction.

A packet refers to a crystal unit in which blocks, which are a collection of laths, are arranged in parallel with each other. Further, the packet is a group of laths whose densest crystal planes are parallel to each other, and one packet refers to a plurality of blocks divided.

In this regard, the long axis refers to an axis along which the martensite packet is extended in the rolling direction, and a short axis refers to an axis aligned in a direction perpendicular to the rolling direction.

The long and short axes are not distinguished from each other as shown in FIG. 2 in the martensite packet that is initially formed before the rolling, but when the packet is rolled, the packet is extended in the rolling direction, forming the long axis in the rolling direction and the short axis perpendicular to the rolling direction.

The long and short axes may be measured by distinguishing the packet on a scanning electron microscope (SEM), and then setting the longest axis of the packet as the long axis and setting the longest axis among axes perpendicular to the long axis as the short axis.

In addition, in martensite included in the steel plate of the present disclosure, an area ratio of packets with a long axis: short axis=2:1 to 20:1 may be 50 to 100%. Preferably, an area ratio of packets with a long axis:short axis length ratio of 5:1 to 20:1 may be 56 to 91%.

As such, the steel plate of the present disclosure not only includes martensite, which is the hard structure, as the matrix structure, but also controls martensite included in the steel plate to have the form that is elongated by the cold rolling, so that the strength of the steel plate and a part manufactured using the same may be more effectively improved.

The steel plate of the present disclosure does not completely exclude inclusion of structures other than martensite. However, because ferrite, pearlite, bainite, retained austenite, and the like are not desirable for securing the strength and the durability, it is necessary to control fractions thereof within a certain range.

The steel plate may include 0 to 10 area% of one or more microstructures of ferrite and retained austenite, with respect to the total 100 area%, and preferably 1 to 5 area%.

In addition, the steel plate may include 0 to 5 area% of one or more microstructures of pearlite and bainite, with respect to the total 100 area%, and preferably 1 to 2 area%.

In addition, the steel plate may include a case in which a total fraction of ferrite, retained austenite, pearlite, and bainite is 0 area%.

In one example, the steel plate of the present disclosure may further include cementite, precipitates, and the like as a residual structure in addition to the aforementioned microstructure, but the present disclosure may not be limited thereto.

The steel plate of the present disclosure satisfies the aforementioned alloy composition and satisfies 90 area% or greater of the martensite microstructure, so that the tensile strength (TS) may be 1800 to 2500 MPa and the yield strength (YS) may be 1700 to 2500 MPa. A preferable tensile strength (TS) may be 1830 to 2200 MPa and a yield strength (YS) may be 1810 to 2100 MPa.

In particular, when the alloy composition of the steel plate satisfies C: 0.18 to 0.30%, the tensile strength (TS) may be equal to or greater than 1910 MPa and the yield strength (YS) may be equal to or greater than 1880 MPa.

The yield strength (MPa) and alloying elements (%) of the steel plate satisfy following Relational Expression 1, so that the present disclosure may secure very high strength without adding a large amount of alloying elements of carbon or manganese.

Generally, to increase the strength of the steel plate, the contents of carbon and manganese are increased, but in this case, the weldability and the formability of the steel plate are reduced. However, the present disclosure exhibits the effect of exhibiting the high strength even with a small content of carbon or manganese by satisfying Relational Expression 1, and there is also an economic advantage in terms of the manufacturing cost.$\left[yield strength/\left\{C+\left(Mn\times 0.05\right)\right\}\right] \geq 6 , 000$

Preferably, 10,100≥[yield strength/{C+(Mn×0.05)}]≥6,000 may be satisfied, and more preferably, 7,800≥[yield strength/{C+(Mn×0.05)}]≥6,000 may be satisfied.

FIG. 1 is a flowchart showing a method for manufacturing a high-strength steel plate according to the present disclosure.

Referring to FIG. 1, the method for manufacturing the steel plate according to the present disclosure may further include heating a slab including, in wt%, C: 0.11 to 0.30%, Mn: 0.10 to 3.00%, Si: greater than 0% and equal to or smaller than 0.50%, Al: greater than 0% and equal to or smaller than 0.10%, P: greater than 0% and equal to or smaller than 0.05%, S: greater than 0% and equal to or smaller than 0.03%, N: greater than 0% and equal to or smaller than 0.03%, remainder Fe and other unavoidable impurities, hot-rolling the heated slab, rapidly cooling the hot-rolled slab at a cooling rate of 50 to 1000°C/sec within 5 seconds after the hot rolling and then coiling the cooled slab, and cold-rolling the slab after the coiling. The steel plate may further include B: 0.0003 to 0.005wt%.

### Slab heating and hot rolling

A slab steel composition of the present disclosure is the same as the steel composition of the steel plate described above, so that it will be omitted. Slab manufacturing conditions may not be particularly limited, and slab manufacturing conditions used for manufacturing general steel plates may be applied.

The prepared slab is heated at 1050 to 1350°C. The slab may be heated in a temperature range equal to or higher than 1100°C for sufficient homogenization treatment. However, when the slab heating temperature is excessively high, it may not only be undesirable in terms of the economic efficiency, but also may have a negative effect on the surface quality of the final product, so that an upper limit of the slab heating temperature may be equal to or lower than 1350°C.

The heated slab may be hot rolled under normal hot rolling conditions, but a finishing rolling temperature may be 800 to 950°C, preferably 850 to 930°C, and more preferably 856 to 930°C, for controlling a rolling load and reducing the surface scale.

### Cooling and coiling

The cooling under rapid cooling conditions may be performed on the hot-rolled steel plate immediately after the hot rolling.

Because the present disclosure aims to strictly control the microstructure of the steel plate, it is preferable that the cooling starts within 5 seconds immediately after end of the hot rolling. This is because, when a time period from the end of the hot rolling to the start of the cooling exceeds 5 seconds, unintended ferrite, pearlite, and bainite may be formed by air cooling in atmosphere. A preferable time period from the end of the hot rolling to the start of the cooling may be greater than 0 seconds and equal to or smaller than 3 seconds.

Considering equipment limitations and economic efficiency, the cooling rate of the hot-rolled steel plate may be adjusted.

The hot-rolled steel plate immediately after the hot rolling may be cooled to a cooling end temperature equal to or lower than 350°C at a cooling rate of 50 to 1,000°C/s, preferably may be cooled to 100 to 300°C at a cooling rate of 100 to 300°C/s, and more preferably may be cooled to 150 to 295°C at a cooling rate of 100 to 300°C/s.

When the cooling end temperature exceeds 350°C, transformation into ferrite, pearlite, and bainite is inevitable, so that the present disclosure may set an upper limit of the cooling end temperature to 350°C to secure the microstructure that the present disclosure aims for. In one example, a lower limit of the cooling end temperature may be equal to or higher than 100°C, and preferably may be equal to or higher than 150°C. When the cooling temperature is lower than 100°C, the transformation into ferrite, pearlite, and bainite occurs during the cooling, so that it may be difficult to secure the microstructure that the present disclosure aims for.

The present disclosure performs the cooling under the rapid cooling conditions on the hot-rolled steel plate immediately after the hot rolling, so that 90 area% or greater of martensite may be secured in the hot-rolled steel plate state before the application of the cold rolling. A typical method for manufacturing the steel plate includes performing the heat treatment immediately after the hot rolling, cold-rolling the heat-treated hot-rolled steel plate, and then performing the quenching heat treatment to form the martensite structure.

However, the present disclosure may exhibit the high-strength steel plate, including 90 area% or greater of martensite, and particularly, 60 area% or greater of elongated martensite, by controlling the alloy composition ratio and the conditions of rapid cooling and cold rolling despite omitting the heat treatment immediately after the hot rolling and the quenching after the cold rolling.

The hot-rolled steel plate after the end of the cooling may be coiled into a hot-rolled coil. A coiling temperature may be equal to or lower than 350°C similar to the cooling conditions, preferably, may be 100 to 300°C, and more preferably, may be 110 to 250 °C.

### Cold rolling

After uncoiling the hot-rolled coil, cold rolling may be performed at a reduction percentage of 50 to 80%.

When the cold rolling reduction percentage is smaller than 50%, sufficient elongation of martensite is not achieved, and thus desired high strength characteristics is not able to be secured. Therefore, regarding a lower limit, the cold rolling reduction percentage may be equal to or greater than 50%, and preferably equal to or greater than 60%.

On the other hand, when the cold rolling reduction percentage exceeds 80%, not only may there be a concern about equipment damage resulted from a rolling load, but there may also be a problem of cracks occurring in the material during the cold rolling. Therefore, regarding an upper limit, the cold rolling reduction percentage may be equal to or smaller than 80%, and preferably, may be equal to or smaller than 75%.

The high-strength steel plate manufactured through the above-described manufacturing method may include 90 volume% or greater of martensite as the microstructure, and may have the tensile strength equal to or greater than 1800 MPa and the yield strength equal to or greater than 1700 MPa.

Specific examples of the high-strength steel plate and the method for manufacturing the same are as follows.

### 1. Manufacturing of high-strength steel plate

After manufacturing slabs having compositions in Table 1 below, steel plate specimens were manufactured by applying process conditions in Table 2 below. Each slab was heated in a temperature range of 1050 to 1350°C and homogenized.

Alloy compositions in Table 1 are identified via a dry analysis method, a wet analysis method, and the like in a cold-rolled steel plate state.

**[Table 1]**

| Steel type | Alloy composition (wt%) | | | | | | | |
|---|---|---|---|---|---|---|---|---|
| | C | Mn | Si | Al | P | S | N | B |
| A | 0.223 | 0.979 | 0.08 | 0.03 | 0.005 | 0.002 | 0.004 | 0.0013 |
| B | 0.126 | 1.09 | 0.05 | 0.04 | 0.009 | 0.003 | 0.003 | 0.0021 |
| C | 0.171 | 1.21 | 0.06 | 0.02 | 0.012 | 0.005 | 0.005 | 0.0018 |
| D | 0.292 | 0.88 | 0.08 | 0.03 | 0.014 | 0.004 | 0.004 | 0.0016 |
| E | 0.219 | 2.8 | 0.07 | 0.02 | 0.011 | 0.003 | 0.005 | 0.0015 |
| F | 0.227 | 1.06 | 0.41 | 0.03 | 0.009 | 0.004 | 0.003 | 0.0041 |
| G | 0.226 | 1.13 | 0.03 | 0.07 | 0.019 | 0.006 | 0.005 | 0.0022 |
| H | 0.102 | 0.99 | 0.07 | 0.02 | 0.012 | 0.006 | 0.004 | 0.0018 |
| I | 0.218 | 1.03 | 0.06 | 0.03 | 0.015 | 0.004 | 0.007 | 0.0002 |
| J | 0.231 | 3.21 | 0.08 | 0.02 | 0.016 | 0.006 | 0.003 | 0.0018 |

**[Table 2]**

| Classificatio n | Stee l type | Rolling end temperatur e (°C) | Coolin g start time (sec) | Coolin g rate (°C/sec ) | Cooling end temperatur e (°C) | Coiling temperatur e (°C) | Cold rolling reduction percentag e (%) |
|---|---|---|---|---|---|---|---|
| 1 | A | 910 | 2.4 | 100 | 294 | 250 | 60 |
| 2 | A | 892 | 2.2 | 200 | 157 | 117 | 60 |
| 3 | A | 886 | 1.6 | 300 | 241 | 216 | 60 |
| 4 | A | 930 | 1.7 | 100 | 250 | 235 | 60 |
| 5 | A | 912 | 2.9 | 100 | 236 | 222 | 60 |
| 6 | A | 921 | 2.2 | 100 | 223 | 194 | 75 |
| 7 | B | 929 | 1.8 | 100 | 259 | 231 | 60 |
| 8 | C | 911 | 1.7 | 100 | 225 | 210 | 60 |
| 9 | D | 895 | 2.2 | 100 | 256 | 217 | 60 |
| 10 | E | 882 | 1.7 | 100 | 218 | 200 | 60 |
| 11 | F | 894 | 1.1 | 100 | 179 | 148 | 60 |
| 12 | G | 856 | 2.2 | 100 | 263 | 238 | 60 |
| 13 | A | 889 | 6.4 | 100 | 199 | 181 | 60 |
| 14 | A | 773 | 2.2 | 100 | 151 | 135 | 60 |
| 15 | A | 905 | 2.4 | 100 | 391 | 359 | 60 |
| 16 | A | 916 | 2.0 | 35 | 201 | 172 | 60 |
| 17 | A | 912 | 2.0 | 100 | 151 | 132 | 45 |
| 18 | H | 921 | 1.2 | 100 | 220 | 204 | 60 |
| 19 | I | 916 | 2.4 | 100 | 188 | 168 | 60 |
| 20 | J | 926 | 1.0 | 100 | 278 | 228 | 60 |

### 2. Materiality evaluation method and results thereof

Thereafter, a microstructure of each specimen was measured, and results thereof are shown in Table 3. Each specimen was cut in a direction parallel to the rolling direction, and then a specimen for observing the microstructure was collected from a cut surface at a 1/4 point of a plate thickness. The specimens collected as such were polished and etched with a nital etchant, and the microstructure of each specimen was observed using an optical microscope and the scanning electron microscope (SEM). A microstructure fraction was measured as an area percentage of each phase in a 200x optical microscope image and 500x and 5000x SEM images.

As for elongated martensite, an area of each martensite packet having a long axis direction parallel to the rolling direction within 45° in the scanning electron microscope image was measured. Additionally, also as for a long-short axis ratio of the martensite packet, an area of each martensite packet having a length ratio of the long axis to the short axis within a range of 2:1 to 20:1 in the scanning electron microscope image was measured.

In Table 3, M represents martensite, F represents ferrite, R-γ represents retained austenite, P represents pearlite, and B represents bainite.

**[Table 3]**

| Clas sific atio n | Microstructure fraction (area%) | | | | | Area percentage (%) of martensite elongated in rolling direction | Area percentage (%) of martensite packet with long-short axis ratio of 2:1 to 20:1 |
|---|---|---|---|---|---|---|---|
| | M | F | R-γ | P | B | | |
| 1 | 98 | 0 | 1 | 0 | 1 | 81 | 91 |
| 2 | 100 | 0 | 0 | 0 | 0 | 80 | 87 |
| 3 | 100 | 0 | 0 | 0 | 0 | 86 | 77 |
| 4 | 98 | 0 | 1 | 0 | 1 | 94 | 75 |
| 5 | 97 | 0 | 1 | 1 | 1 | 84 | 67 |
| 6 | 99 | 0 | 1 | 0 | 0 | 91 | 77 |
| 7 | 95 | 0 | 0 | 2 | 3 | 83 | 75 |
| 8 | 95 | 1 | 0 | 2 | 2 | 88 | 81 |
| 9 | 100 | 0 | 0 | 0 | 0 | 95 | 70 |
| 10 | 98 | 0 | 2 | 0 | 0 | 81 | 86 |
| 11 | 100 | 0 | 0 | 0 | 0 | 80 | 75 |
| 12 | 100 | 0 | 0 | 0 | 0 | 85 | 81 |
| 13 | 88 | 11 | 0 | 0 | 1 | 75 | 74 |
| 14 | 88 | 6 | 0 | 4 | 2 | 78 | 69 |
| 15 | 85 | 0 | 3 | 0 | 12 | 72 | 59 |
| 16 | 85 | 1 | 1 | 4 | 9 | 84 | 72 |
| 17 | 100 | 0 | 0 | 0 | 0 | 56 | 48 |
| 18 | 68 | 24 | 0 | 4 | 4 | 58 | 56 |
| 19 | 69 | 22 | 0 | 5 | 4 | 83 | 78 |
| 20 | 85 | 0 | 15 | 0 | 0 | 81 | 74 |

FIG. 2 is a photograph showing a 100 area% martensite microstructure before cold rolling according to the present disclosure. Referring to FIG. 2, it may be identified that the steel plate includes martensite, the hard structure, as the matrix structure.

FIG. 3 is a photograph showing a martensite microstructure after cold rolling with a 70% reduction percentage according to the present disclosure. Referring to FIG. 3, it may be identified that martensite included in the steel plate has the form that is elongated by the cold rolling.

However, because FIG. 3 is a high-magnification measurement of the martensite packet, it is difficult to measure the long and short axes of the packet from FIG. 3.

A tensile strength and a yield strength for each specimen were measured via a test according to the JIS-5 standard, and results thereof are shown in Table 4.

**[Table 4]**

| Classif ication | Tensile strength (MPa) | Yield strength (MPa) | Yield strength/(C+Mn*0.05) |
|---|---|---|---|
| 1 | 1947 | 1912 | 7031 |
| 2 | 1975 | 1925 | 7077 |
| 3 | 2015 | 1910 | 7024 |
| 4 | 1994 | 1957 | 7195 |
| 5 | 1917 | 1911 | 7027 |
| 6 | 2080 | 2047 | 7526 |
| 7 | 1839 | 1811 | 10034 |
| 8 | 1905 | 1876 | 8104 |
| 9 | 2122 | 2067 | 6152 |
| 10 | 2133 | 2088 | 6824 |
| 11 | 2032 | 2028 | 7244 |
| 12 | 2054 | 2023 | 7162 |
| 13 | 1546 | 1418 | 5214 |
| 14 | 1755 | 1595 | 5865 |
| 15 | 1757 | 1624 | 5972 |
| 16 | 1715 | 1588 | 5839 |
| 17 | 1738 | 1616 | 5941 |
| 18 | 1539 | 1341 | 8851 |
| 19 | 1666 | 1548 | 5744 |
| 20 | 1992 | 1853 | 4733 |

As shown in Tables 1 to 4, Specimens 1 to 12, which satisfy both the alloy composition and the manufacturing conditions of the present disclosure, show a martensite fraction of 95 to 100 area% and a ratio of martensite elongated in the rolling direction of 72 to 95%. In addition, it may be identified that a ratio of martensite packets with a long-short axis ratio of 2:1 to 20:1 is 56 to 91%.

In addition, it may be identified that Specimens 1 to 12 show a tensile strength of 1,839 to 2,133 MPa and a yield strength of 1,811 to 2,088 MPa, and the yield strength and the ratio of alloying elements both satisfy Relational Expression 1.

In terms of the carbon content, Specimens 1 to 6 and Specimens 9 to 12 satisfy the alloy composition of the steel plate of C: 0.18 to 0.30%, and Specimens 7 and 8 satisfy C: smaller than 0.18%. Specimens 1 to 6 and Specimens 9 to 12 show further improved tensile strength and yield strength compared to Specimens 7 and 8.

On the other hand, it may be identified that Specimens 13 to 20, which do not satisfy at least one of the alloy composition and the manufacturing conditions of the present disclosure, do not satisfy at least one of the fraction of martensite, the ratio of martensite elongated in the rolling direction, and the ratio of martensite packets having the long-short axis ratio equal to or greater than 2:1, which are proposed by the present disclosure.

Specimen 13 is a specimen in which the cooling was started 5 seconds after the end of the rolling. It may be identified that desired strength and durability are not secured in Specimen 13 because of a high fraction of ferrite.

Specimen 14 is a case in which the rolling end temperature is low, and Specimen 16 is a case in which the cooling rate is low. It may be identified that the martensite fraction that the present disclosure aims for is not secured and the aimed strength is not secured in these Specimens because of high fractions of pearlite and bainite.

Specimen 15 is a case in which the cooling end temperature and the coiling temperature are high. It may be identified that the aimed strength is not secured in Specimen 15 because of the high fraction of bainite.

Specimen 17 is a case in which the cold rolling reduction rate is low. It may be identified that the aimed strength is not secured in Specimen 17 because of low fraction of elongated martensite and ratio of martensite packets with the long-short axis ratio equal to or greater than 2:1.

Specimen 18 is a case in which the carbon (C) content is low, and Specimen 19 is a case in which the boron (B) content is low. It may be identified that aimed levels of strength and durability are not secured in these Specimens because of significantly low fractions of martensite.

Specimen 20 is a case in which the manganese (Mn) content is high. Because the transformation into martensite did not occur sufficiently, a large amount of residual austenite was formed. It may be identified that Specimen 20 has excellent tensile strength and yield strength because of the high manganese content, but has low efficiency of the alloying elements because the yield strength and the ratio of the alloying elements do not satisfy Relational Expression 1.

Therefore, the high-strength steel plate of the present disclosure has the excellent tensile strength and yield strength, including 90 area% or greater of hard martensite, by lowering the carbon and/or manganese content and controlling the alloy composition ratio and the conditions of the rapid cooling and the cold rolling, despite the omission of the heat treatment immediately after the hot rolling and immediately after the cold rolling.

In particular, because martensite included in the steel plate is controlled to have the elongated form by the cold rolling, the strength of the steel plate and the part manufactured using the same may be more effectively improved.

Although the present disclosure has been described with reference to the accompanying drawings, the present disclosure is not limited by the embodiments disclosed herein and the drawings, and it is obvious that various modifications may be made by those skilled in the art within the scope of the technical idea of the present disclosure. In addition, although the effects based on the configuration of the present disclosure are not explicitly described and illustrated in the description of the embodiment of the present disclosure above, it is natural that predictable effects of the corresponding configuration should also be recognized.

## Claims

1. A steel plate comprising, in weight%, C: 0.11 to 0.30%, Mn: 0.10 to 3.00%, Si: greater than 0% and equal to or smaller than 0.50%, Al: greater than 0% and equal to or smaller than 0.10%, P: greater than 0% and equal to or smaller than 0.05%, S: greater than 0% and equal to or smaller than 0.03%, N: greater than 0% and equal to or smaller than 0.03%, remainder Fe and other inevitable impurities,
wherein the steel plate has a martensite microstructure of 90 to 100 area% with respect to a total 100 area%.

2. The steel plate of claim 1, further comprising B: 0.0003 to 0.005wt%.

3. The steel plate of claim 1, wherein when a packet of the martensite having a long axis direction aligned within 45° from a rolling direction is called martensite elongated along the rolling direction, an area percentage of the martensite elongated along the rolling direction in the martensite is equal to or greater than 60%.

4. The steel plate of claim 1, wherein an area percentage of packets having a long axis to a short axis ratio equal to or greater than 2:1 in the martensite is equal to or greater than 50%.

5. The steel plate of claim 1, wherein the steel plate includes 0 to 10 area% of microstructures of one or more of ferrite and retained austenite with respect to the total 100 area%.

6. The steel plate of claim 1, wherein the steel plate includes 0 to 5 area% of microstructures of one or more of pearlite and bainite with respect to the total 100 area%.

7. The steel plate of claim 1, wherein a tensile strength is equal to or greater than 1800 MPa and a yield strength is equal to or greater than 1700 MPa.

8. The steel plate of claim 1, wherein when C is in a range of 0.18 to 0.30%, a tensile strength is equal to or greater than 1910 MPa and a yield strength is equal to or greater than 1880 MPa.

9. The steel plate of claim 1, wherein a yield strength (MPa) and alloying elements (%) of the steel plate satisfy following Relational Expression 1.$\left[yield strength/\left\{C+\left(Mn\times 0.05\right)\right\}\right] \geq 6 , 000$

10. A method for manufacturing a steel plate, the method comprising:
(a) heating a slab including, in wt%, C: 0.11 to 0.30%, Mn: 0.10 to 3.00%, Si: greater than 0% and equal to or smaller than 0.50%, Al: greater than 0% and equal to or smaller than 0.10%, P: greater than 0% and equal to or smaller than 0.05%, S: greater than 0% and equal to or smaller than 0.03%, N: greater than 0% and equal to or smaller than 0.03%, remainder Fe and other unavoidable impurities;
(b) hot-rolling the heated slab;
(c) rapidly cooling the hot-rolled slab at a cooling rate of 50 to 1000°C/sec within 5 seconds after the hot rolling and then coiling the cooled slab; and
(d) cold-rolling the slab after the coiling.

11. The method of claim 10, wherein in the (a), the heating is performed at 1050 to 1350°C.

12. The method of claim 10, wherein in the (b), the hot rolling is performed at 800 to 950°C.

13. The method of claim 10, wherein in the (c), each of the rapid cooling and the coiling is performed at 100 to 350°C.

14. The method of claim 10, wherein in the (d), the cold rolling is performed at a reduction percentage of 50 to 80%.
